

Nov. 12, 1946.

A. T. PETERS

2,410,837

### CAST INGOT

Filed April 17, 1944

4 Sheets-Sheet 1



Fig. 1

INVENTOR.  
*Adolph T. Peters*

BY

*Griswold & Burdick*  
ATTORNEYS

Nov. 12, 1946.

A. T. PETERS

2,410,837

CAST INGOT

Filed April 17, 1944

4 Sheets-Sheet 2



INVENTOR.  
Adolph T. Peters

BY

Griswold & Burdick  
ATTORNEYS

Nov. 12, 1946.

A. T. PETERS

2,410,837

CAST INGOT

Filed April 17, 1944

4 Sheets-Sheet 3



Fig. 4



INVENTOR.  
Adolph T. Peters

Griswold & Burdick  
ATTORNEYS

Fig. 5

Nov. 12, 1946.

A. T. PETERS

2,410,837

CAST INGOT

Filed April 17, 1944

4 Sheets-Sheet 4



*Fig. 6*



*Fig. 7*



*Fig. 8*



*Fig. 9*

Inventor  
Adolph T. Peters

By

Griswold & Burdick  
Attorneys

Patented Nov. 12, 1946

2,410,837

# UNITED STATES PATENT OFFICE

2,410,837

## CAST INGOT

Adolph T. Peters, Midland, Mich., assignor to The Dow Chemical Company, Midland, Mich., a corporation of Michigan

Application April 17, 1944, Serial No. 531,313

7 Claims. (Cl. 22—200.1)

1

The invention relates to cast metal. It more particularly concerns improved cast ingot and a method of and means for casting the same of alloyed magnesium, the liquidus of which passes through a wide range of temperature as it solidifies.

Wide freezing range magnesium alloys, particularly those used for structural purposes, generally solidify in two principal phases, a solid solution which constitutes the major portion of the solid metal and an intermetallic compound formed between magnesium and the principal alloying constituent, comprising the balance. Attempts to cast such alloys in ingot form have heretofore yielded a product lacking in uniformity of composition as regards the average concentration of alloying constituents from point to point throughout the ingot and having an undesirable metallographic structure particularly as regards the particle size and distribution of the second phase throughout the solid solution phase and the nature of the distribution of the dissolved constituent in the same solid solution phase. The maldistribution of the alloying metal and particle size of the second phase is responsible, in considerable measure, for the undesirable variations in physical properties developed in wrought products formed from conventional ingots of alloyed magnesium.

A particular object is to provide an alloyed magnesium ingot yielding superior wrought metal on being mechanically deformed thereinto as by forging, rolling, and extrusion.

Another object is to provide a method of casting ingot of the aforesaid character in a continuous length.

Another object is to provide an apparatus suitable for casting wide freezing range metal in a continuous length.

Other objects and advantages will appear as the description proceeds.

The term "freezing range," as used herein and in the appended claims, means the difference between the temperature of the molten alloy when solid metal first appears on cooling the same and the temperature of the alloy when it has just entirely solidified from the molten state under equilibrium conditions. The term "liquidus" refers to the curve relating the temperature and composition of the liquid portion of the alloy as it is cooled through the freezing range in contact with the solid portion of the alloy thereby deposited from the liquid; and the term "solidus" refers to the curve relating the temperature and composition of the solid metal so deposited. The lower

5 temperature of the freezing range so defined is the melting point of the lowest melting eutectic if such exists. Molten magnesium alloy having a temperature above the maximum of the freezing range contains "superheat" and is referred to herein as "superheated."

10 My invention is predicated upon the discovery that by cooling the upper end of the preformed ingot of alloyed magnesium, the alloy having a wide freezing range, positioned adjacent to the larger end of a shallow mold, the inside tapering inwardly from the bottom; adding to the mold molten superheated alloyed magnesium having a wide freezing range while preventing loss of heat therefrom through the mold wall so as to maintain a pool of liquid metal therein turning to slush at the bottom thereof in contact with the cooled ingot as heat from the slush is removed substantially wholly by conduction through the 15 ingot, slush being thereby molded to the form of the ingot and then frozen thereto to increase its length, the unfrozen portion of the slush acting to seal the mold against escape of liquid metal between the frozen slush and the mold wall; lowering the so lengthened ingot at a rate equivalent to the rate at which such increase in length occurs and in alignment with the mold so as to withdraw from the mold slush as it is molded, sound ingot is obtained having a unique metallographic structure and substantial uniformity of composition throughout its length and breadth adapted for 20 mechanical deformation into wrought products possessing superior strength properties.

25 The invention then consists in the ingot, method, and apparatus hereinafter fully described and particularly pointed out in the claims, the annexed drawings and the following description setting forth certain means and mode of carrying out the invention.

In the said annexed drawings:

Fig. 1 is a side elevation partly in section of an embodiment of the ingot casting apparatus showing ingot being cast from slush metal in a metal holder or mold.

45 Fig. 2 is a similar view showing a portion of the apparatus of Fig. 1 arranged for starting its operation with a dummy block.

Fig. 3 is a similar view of a portion of Fig. 1 showing the formation of slush in the metal holder on top of the dummy block as pouring of ingot is commenced.

50 Fig. 4 is a similar view of a portion of Fig. 1 showing a short section of ingot formed on the dummy block.

Fig. 5 is a similar but enlarged fragmentary

2

view of a portion of Fig. 1 showing in detail the transformation of liquid metal into slush, molding it to the form of ingot, and freezing the same into solid ingot in continuous sequence.

Fig. 6 is a photomicrograph, at 100 diameters, showing the metallographic structure of Dow-metal J-1, cylindrical 13-inch diameter ingot, taken at a point 1 inch from the cylindrical surface in a plane perpendicular to the axis, the ingot being cast in accordance with the invention.

Fig. 7 is a similar photomicrograph to Fig. 6, taken 3 inches from the cylindrical surface of the ingot.

Fig. 8 is a similar photomicrograph to Fig. 6, taken on the axis of the ingot.

Fig. 9 is a similar photomicrograph to Fig. 6 but more deeply etched, revealing coring of the solid solution phase, magnification 200 diameters.

In the several figures like numerals refer to like parts.

Referring to the drawings, numeral 10 is a vertically disposed metal holder or mold, open at the top and bottom, for molten metal and slush formed thereof. The inside wall of the mold slopes inwardly from the bottom 11 which is the larger end of the mold and opens downwardly. The metal holder is provided with means to preclude loss of heat, such as a covering of thermal insulation 12. If desired, a thin metal ring 26 is attached close to the bottom of the mold to hold the insulation in place. The rim 13 is attached to the top of the mold 10 and rests upon a support 14 carried on legs 15 and 16. Means for imparting vibration to the mold, such as an air operated vibrator 17, is shown mounted on the beam 18 carried by supports 19 and 20, the lower ends of which are attached to diametrically opposite points 21 and 22, respectively, on the rim 13.

Means are provided for bringing molten metal to the metal holder such as the tilting ladle 23 carried by bail 24 which is shown in Fig. 1 resting upon the hook 25, although other means may be used, such as a siphon or liquid metal pump, delivering molten metal to the holder or mold through a pipe.

A cooling water launder 27, such as one having a right triangular cross-section, is arranged adjacent to the bottom of the metal holder. Extending around the inner circumferential face 28 of the launder are parallel rows of uniformly spaced small holes 29, drilled perpendicularly to the face 28 and thereby forming jets directed at an angle, such as 45°, to the vertical. The launder is provided with a cooling water connection 30 to a valved water supply 31.

Guide wheels 32 and 33 are arranged so that their treads 34 and 35, respectively, are in vertical alignment with the inner circumference of the larger end 11 of the metal holder. Driving wheel 36 has a tread 37 in vertical alignment with a diametrically opposite point on the inner circumference of the metal holder from that of the treads of guide wheels 32 and 33. The driving wheel 36 is rotated by worm gear 38 operated by worm pinion 39 driven through reduction gear 40 by motor 41 provided with speed regulation controls 42.

In starting the process, a dummy block 43 of suitable length and having the cross-sectional form of the ingot to be cast, is positioned against the treads 34 and 35 of the guide wheels 32 and 33 and the tread 37 of the driving wheel 36, with which it frictionally engages, so that the con-

cave head 44 engages the bottom end 11 of the liquid metal and slush holder 10 to form a bottom closure therefor, as shown particularly in Fig. 2. The dummy block is preferably made by casting a length of ingot in the usual manner or otherwise of a magnesium alloy having a similar composition to that to be cast, although other metals may be used.

Cooling water is directed against the dummy block by opening the valve in the cooling water supply line 31 thereby providing a curtain of water 45 from the jets 29 drenching the vertical surface of the block. In so drenching the surface of the ingot, it is desirable that the water be directed downwardly at an angle to the vertical, as with the apparatus provided, so that the water is uniformly distributed and directed away from contact with the bottom 11 of the metal holder 10.

While the dummy block is thus cooled molten magnesium alloy to be cast into ingot and containing a sufficient amount of superheat is introduced into the metal holder 10 from the top, as by ladling in the manner indicated in Fig. 1, to a depth approaching the brim 13 of the metal holder 10. The average temperature of the wall of the metal holder or mold is maintained above the temperature of the liquidus of the alloy in the mold by the superheat of the liquid metal introduced thereinto, loss of heat from the mold being precluded by insulation 12, or by the use of an external heater around the mold (not shown), so as to prevent the formation of solid alloy particles by abstraction of latent heat through the mold wall. Since the metal holder 10 is insulated, as with the insulation 12, or otherwise made proof against substantial heat loss, heat from the liquid metal (i. e. superheat of the liquid and latent heat) immediately begins to be conducted away substantially wholly through the head 44 into the cooled dummy block 43. The effect of such heat transfer is to bring about crystallization of solid metal within the liquid to form therewith a bed of slush 47 of solid metal particles mixed with liquid metal supported by the wall of the mold and the top of the dummy block as shown in Fig. 3.

The slush bed thus formed is of gradually decreasing density (i. e. ratio of volume of solid metal particles to that of liquid) toward the supernatant liquid metal 48. The slush adjacent to the top of the dummy block becomes increasingly dense as the liquid therewith cools until it all freezes. I have found that as this slush becomes increasingly dense, it passes through a stage in which it is moldable and use is made of this property in my process by shaping or molding the slush to the cross-sectional form of the ingot desired before final freezing occurs. This shaping is accomplished adjacent to the big inwardly tapered end 11 where the slush approaches its maximum density and takes the cross-sectional form of the opening of the mold before final freezing of the entrained liquid alloy occurs.

The slush thus shaped is lowered from the mold by lowering the dummy block thereby bringing a further quantity of slush into molding position. While the molded slush is being thus lowered, the liquid therein freezes forming of the slush a solid body of metal having the cross-section of the ingot desired. A portion of ingot 50 thus produced is shown in Fig. 4, resting on the top 44 of the dummy block 43, the line of demarkation between the frozen and unfrozen slush being indicated at 48. The unfrozen slush also acts to

seal the bottom of the metal holder against leakage of the supernatant liquid metal 48, the depth of which is kept shallow so as to minimize the liquid pressure head on the slush. Complete solidification of the metal into ingot is thus brought about below or just inside the bottom of the mold or holder 10, the temperature of the wall thereof being maintained by the liquid metal introduced above the lowest temperature reached on the liquidus curve when the liquid metal is all just frozen, usually the eutectic melting point.

In carrying out the method in continuous manner, after forming a body of slush 47 as described, the dummy block 43 is lowered continuously at a rate such that only the relatively dense molded slush emerges from the metal holder, the balance of the slush slumping downwardly, forming a seal while liquid metal is added, preferably at a substantially constant rate, so as to maintain its level and the inventory of slush therein, at a substantially constant shallow depth. Too rapid lowering of the slush through the big end 11 is revealed by a loss of the sealing action, while, if the lowering is too slow, the lower portion of the slush tends to freeze to a completely solid mass within the metal holder, hindering lowering. Regulation of the rate of lowering of the dummy block, and the ingot metal which follows it, as the operation proceeds, as shown in Fig. 3, is accomplished by adjusting the speed of the motor 41 with controls 42. The speed of the driving wheel 36 is thereby adjusted to the proper value. The proper speed varies primarily with the alloy composition, initial temperature (extent of super-heating) of the liquid metal, diameter of the cast ingot, and temperature and volume of cooling water and is readily ascertained by trial. As an illustration, in casting 12-inch diameter ingot of "Dowmetal O" (nominally composed of 8.5 per cent aluminum, 0.2 per cent manganese, and 0.5 per cent zinc, the balance being magnesium), using a pouring temperature of 1260° F. (i. e. temperature at which the metal is introduced into the metal holder) in a frusto-conical metal holder tapering inwardly from the bottom at the rate of  $\frac{1}{4}$  inch per foot, and having a depth of 8 inches, formed of  $\frac{1}{4}$  inch boiler plate surrounded by 1 inch thick asbestos thermal insulation, and using about 20 gallons per minute of cooling water at 45° F., a suitable rate of lowering is between about 2.0 and about 2.7 inches per minute, about 2.5 inches being preferred.

As the operation proceeds, cohesion between the solid metal particles and the ingot is largely relied upon to move the slush downwardly through the metal holder 10, which molds the slush as it passes therethrough, however, some of the metal particles in the slush may tend to stick to the mold surface, necessitating the provision of means to dislodge them as by the use of a vibrator (air hammer), such as that shown as 17 in Fig. 1, which vibrates or preferably imparts a continuous series of sharp blows to the metal holder. I have found that by making the total depth of the slush and supernatant liquid metal between about 5 inches and 9 inches and preferably about 7 inches, using a metal holder tapering inwardly from the bottom at a rate between about  $\frac{1}{8}$  inch and  $\frac{3}{4}$  inch per foot, continuous downward movement of the slush is readily obtained using vibrations at the rate of 20 per second and an amplitude of not over about 0.07 inch or a series of sharp blows at one second intervals moving the mold rapidly a distance not over about 0.07 inch. In such operation, the depth of the slush bed

may be from about 1 to 2 inches and the height of the upper edge of the solidified ingot 50 may be as high as 1 inch inside the bottom of the metal holder or as low as  $\frac{1}{4}$  inch below the same, this height being controlled by suitably regulating the rate of lowering the formed ingot as aforesaid. In Fig. 5, the molded slush emerging below the mold as the slush slumps therein is indicated at 51 adjacent to the frozen top edge 52 of the ingot, as when the process is operated so that final freezing of the ingot occurs wholly outside or below the mold.

Ingot 50 formed in this manner may be increased in length as much as desired. In Fig. 1, the ingot is shown increased in length to below the guide wheel 33 with the dummy block still attached. This may be cut off, as with a traveling saw (not shown), and the ingot cut in a similar manner into convenient lengths, if desired, as ingot is produced.

The method may be practiced with any of the magnesium-base alloys, the liquidus curve of which extends over a substantial range of temperature and composition as the alloy solidifies. This is the case with the alloys of magnesium usually used for the manufacture of extrusions, forgings, rolled and drawn products, which have a freezing range of more than 125 Fahrenheit degrees. Such alloys usually contain aluminum, as the principal solid solution and intermetallic compound forming alloying ingredient, in amount between about 3 per cent and 10 per cent, although, in some cases, the aluminum content may be as high as 12 per cent or more. Zinc also forms solid solutions and sometimes intermetallic compounds with magnesium and may be present in the alloys in amount between about 0.5 and 3 per cent or more, either as the sole alloying agent or in combination with other alloying constituents, particularly aluminum. In the magnesium-base alloys containing both aluminum and zinc as alloying constituents in the aforesaid amounts, the solid solution contains most of the aluminum and substantially, if not all, the zinc, the balance of the aluminum and zinc, if any, forming intermetallic compound. Manganese in small amount, e. g. 0.1 to 0.3 per cent, is generally added to the magnesium alloys to enhance corrosion resistance and it does not substantially affect the freezing range. Examples of such alloys containing aluminum, zinc, and manganese are given in the accompanying table, together with the freezing temperature, that is, the temperature at which solid particles begin to deposit and form slush as the molten alloy is slowly cooled, as under equilibrium conditions. Temperatures which are 125 to 250 Fahrenheit degrees or more below the freezing temperature are usually required to completely solidify these alloys.

Table I

| Dowmetal alloy   | Nominal composition, percent |     |     |         | Freezing temp., ° F. |
|------------------|------------------------------|-----|-----|---------|----------------------|
|                  | Al                           | Mn  | Zn  | Mg      |                      |
| FS and FS-1..... | 3.0                          | 0.3 | 1.0 | Balance | 1,160                |
| J and J-1.....   | 6.5                          | 0.2 | 1.0 | do      | 1,145                |
| O and O-1.....   | 8.5                          | 0.2 | 0.5 | do      | 1,130                |

By thus manipulating the slush so as to mold it as it is formed, substantially wholly abstracting its heat through the ingot into which it solidifies, and regulating the rate of lowering of the slush so that the solidification occurs adjacent the bottom of the mold, preferably substantially wholly below the mold, a unique metallographic struc-

ture results in the ingot. This structure is characterized by (1) substantially uniform but small sized masses of cored solid solution phase of one or more alloying constituents in magnesium and (2) a second phase which is generally an intermetallic compound of magnesium and the principal alloying ingredient (e. g. Mg<sub>17</sub>Al<sub>12</sub> in magnesium-base alloys containing aluminum as the principal alloying metal) in exceedingly small particles having a maximum width of 0.0006 inch distributed through the solid solution phase. In Figs. 6, 7, and 8, the intermetallic compound is shown as small light particles having widths of up to about 0.0004 inch surrounded by a dark line of demarkation, the remaining light background being the cored solid solution phase. In Fig. 9, the background of cored solid solution phase is accentuated by the deeper etch. This reveals the aluminum concentration gradient in the cored solid solution phase, the aluminum concentration being greatest adjacent the particles of the intermetallic compound.

As regards uniformity of composition, typical analysis of representative samples from scalped 12-inch diameter Dowmetal J-1 ingot cast, in accordance with the invention, and sampled at the center line, and at 3 inches, and 6 inches therefrom in a plane perpendicular to the axis, show an aluminum concentration of 6.5 per cent, 6.6 per cent, and 6.6 per cent, respectively. Similar samples taken from adjacent sections of the ingot showed similar values for the aluminum concentration. The variations in the aluminum concentration in ingot similarity cast in other magnesium-base alloys do not exceed the foregoing and all such variations are less than about 2 per cent of the total amount of alloying ingredient from place to place throughout the ingot, the size of the sample being large enough, e. g. 5 to 10 grams, to be representative. In comparison with this, similar sampling of conventional 12-inch diameter ingot of the same alloy cast in 30-inch lengths gave aluminum concentrations varying both from the center toward the outside and from top to bottom, the variations from top to bottom, respectively, being from 6.0 per cent to 6.8 per cent along the axis, 6.4 per cent to 6.8 per cent 3 inches from the axis, and 6.6 per cent to 6.7 per cent 6 inches from the axis. As regards the uniformity of distribution of manganese, that of the ingot of the invention showed no significant variation from center to outside and lengthwise of the ingot, while the concentration in conventional ingot varied from a minimum of 0.16 per cent to a maximum of 0.33 per cent.

By virtue of the unique metallographic structure, especially the uniform distribution and smallness of the particle size of the second phase, even spacing and sharp concentration gradient of the coring of the solid solution phase, and uniformity of composition, the ingot has its principal utility as stock material for making wrought products such as extrusions.

In such uses, an important advantage is that the extruded product not only exhibits high values for strength properties but also greater uniformity of properties from point to point throughout the extrusion compared to extrusions made from conventionally cast ingot. For example, Dowmetal J-1 cast into 8-inch diameter cylindrical ingot, in accordance with the method described, in which the second phase was in the form of particles having a maximum width of 0.0004 inch distributed between evenly spaced adjacent masses of cored solid solution, was extruded into

a rectangular bar  $\frac{1}{2}$  by 6 inches in cross-section and the tensile and compression properties of the extrusion measured. For the extrusion, a 16-inch length of the cast ingot was heated to 600° Farenheit, placed in the heated container of an extrusion press having a die opening of  $\frac{1}{2}$  inch by 6 inches, and then extruded at the rate of five feet per minute, thereby forming a bar 18 feet long. Tensile strength properties of specimens cut from the extruded bar at 3 $\frac{1}{2}$  feet, 8 $\frac{1}{2}$  feet, and 15 feet from the end first issuing from the die, measured in the direction parallel to the direction of extrusion are tabulated in Table II.

Table II

| Testpiece<br>feet distance<br>from die | Longitudinal strength in thousands of pounds<br>per square inch |          |                                     |                      |
|----------------------------------------|-----------------------------------------------------------------|----------|-------------------------------------|----------------------|
|                                        | Yield <sup>1</sup>                                              | Ultimate | Per cent<br>elongation <sup>2</sup> | Compression<br>yield |
| 3.5                                    | 26.8                                                            | 44.2     | 13.0                                | 23.9                 |
| 8.5                                    | 27.2                                                            | 45.2     | 14.2                                | 25.1                 |
| 15.0                                   | 27.2                                                            | 45.6     | 14.2                                | 25.1                 |

<sup>1</sup> At 0.2 per cent deviation from the modulus line.  
<sup>2</sup> In 2 inches.

For comparison, the properties of similar test pieces cut from the same size bar extruded similarly but from conventionally cast ingot are tabulated in Table III.

Table III

| Testpiece<br>feet distance<br>from die | Longitudinal strength in thousands of pounds<br>per square inch |          |                                     |                      |
|----------------------------------------|-----------------------------------------------------------------|----------|-------------------------------------|----------------------|
|                                        | Tensile                                                         |          |                                     | Compression<br>yield |
|                                        | Yield <sup>1</sup>                                              | Ultimate | Per cent<br>elongation <sup>2</sup> |                      |
| 3.5                                    | 22.5                                                            | 41.4     | 13.7                                | 20.0                 |
| 8.5                                    | 23.2                                                            | 42.7     | 15.5                                | 19.1                 |
| 15.0                                   | 25.6                                                            | 44.5     | 15.0                                | 18.3                 |

<sup>1</sup> and <sup>2</sup>—see Table II.

While the invention has been illustrated with the use of a mold having a circular cross-section (frusto-conical) other shapes may be used such as those of rectangular cross-section or those formed of combinations of plane and curved walls, as an oblong section with rounded sides. In all such molds the inside is made to slope inwardly from the bottom with a substantial taper, such as  $\frac{1}{8}$  inch to  $\frac{3}{4}$  inch per foot, as aforesaid, the taper exceeding the slope required merely for relieving frictional resistance as employed in conventional molds.

Among the advantages of the method are that oxidation of the ingot surface, which occurs between the ingot and mold wall in conventional continuous casting, is obviated as the mold is so filled with metal below the liquid line that air cannot attack the metal surface adjacent to the mold. Also, the interior of the mold wall below the liquid level is not subject to severe abrasion since substantially only either liquid or slush is present in the mold. In addition, the ingot does not suffer from the defects which result from contact with the wall of the mold common in conventional continuous casting. For this reason, also, sticking of the ingot to the mold is obviated.

I claim:

1. The method of casting ingot of alloyed magnesium having a wide freezing range which comprises continuously supplying the molten alloy

to a vertically disposed mold, the inside of said mold sloping inwardly from the bottom, while continuously lowering ingot from below the mold; drenching the sides of the ingot with a coolant so as to carry away heat from the metal supplied to the mold thereby to form a bed of slush therein of liquid metal mixed with solid metal particles, the lower portion of the bed adjacent to the upper end of the ingot freezing thereto and increasing its length; and regulating the rate of lowering of the ingot so that the unfrozen portion of the slush in contact with the ingot is maintained adjacent to the bottom of the mold forming a seal with the mold preventing leakage of liquid metal therefrom.

2. The method of casting ingot of alloyed magnesium having a wide freezing range which comprises continuously supplying the molten alloy to a vertically disposed thermally insulated mold at a rate such that a substantially constant level of liquid metal is established therein, the inside wall of said mold sloping inwardly from the bottom, while lowering ingot from below and in line with the mold; drenching with a coolant the sides of the ingot as it is lowered so as to carry away heat from the metal supplied to the mold thereby to form a bed of slush therein of liquid metal mixed with solid metal particles, the portion adjacent to the upper end of the ingot freezing thereto and increasing its length, the unfrozen portion forming a seal between the mold and the frozen slush preventing escape of liquid metal from the mold; and regulating the rate of lowering of the ingot so that the freezing of the slush onto the end of the ingot occurs substantially wholly below the mold while maintaining the aforesaid seal.

3. The method of casting ingot of alloyed magnesium having a freezing range of more than 125 Fahrenheit degrees which comprises continuously supplying the molten alloy to a vertically disposed mold, the inside wall of said mold sloping inwardly from the bottom at a rate of about  $\frac{1}{8}$  to  $\frac{3}{4}$  inch per foot while continuously lowering ingot from below the mold; drenching the sides of the ingot with a coolant so as to carry away heat from the metal supplied to the mold thereby to form a body of slush therein of liquid metal mixed with solid metal particles, the lower portion adjacent to the upper end of the ingot freezing thereto and increasing its length; and regulating the rate of lowering of the ingot so that the freezing of the slush onto the end of the ingot occurs substantially wholly below the mold, the unfrozen portion of the slush forming a seal between the mold and the frozen slush thereby to prevent escape of liquid metal from the mold.

4. The method of casting ingot of alloyed magnesium having a freezing range of more than 125 Fahrenheit degrees which comprises continuously supplying the molten alloy to a vertically disposed thermally insulated mold, the inside wall of said mold sloping inwardly from the bottom at the rate of from  $\frac{1}{8}$  to  $\frac{3}{4}$  inch per foot, while continuously lowering ingot from below the mold; vibrating the mold; drenching the sides of the ingot with a coolant so as to carry away heat from the metal supplied to the mold thereby to form a bed of slush therein of liquid metal mixed with metal particles, the portion of the bed adjacent to the upper end of the ingot freezing solid thereto and increasing its length; and regulating the rate of lowering of the ingot so that the freezing of the slush into ingot occurs substantially wholly below the mold.

5. In a method of casting ingot of alloyed magnesium in a continuous length, the steps which consist in cooling a section of the precast ingot near one end thereof; positioning the cooled end adjacent to the bottom of a vertically disposed mold insulated against substantial heat loss and having insides sloping inwardly from the bottom; introducing molten magnesium alloy into the mold so as to maintain a pool of liquid metal at a substantially constant level therein, thereby cooling the alloy by transferring heat to the cooled end of the ingot and forming a body of slush of solid metal particles mixed with liquid metal beneath the pool, the slush adjacent to the ingot conforming to the shape of the mold and freezing onto the end of the ingot to form an extension thereof, and the unfrozen slush forming a seal preventing the liquid metal from escaping from the mold between it and the extension of the end of the ingot; and lowering the ingot at a rate sufficient to compensate for the extension thus produced so as to maintain its position just below the mold without breaking the seal formed by the slush.
- 10 6. In a method of casting ingot of alloyed magnesium in a continuous length, the steps which consist in cooling a section of the precast ingot near one end thereof; positioning the cooled end adjacent to the bottom of a vertically disposed mold insulated against substantial heat loss and having insides sloping inwardly from the bottom; introducing molten magnesium alloy into the mold so as to maintain a pool of liquid metal at a substantially constant level therein, thereby 15 cooling the alloy by transferring heat to the cooled end of the ingot and forming a body of slush of solid metal particles mixed with liquid metal beneath the pool, the slush adjacent to the ingot conforming to the shape of the mold and freezing onto the end of the ingot to form an extension thereof, and the unfrozen slush forming a seal preventing the liquid metal from escaping from the mold between it and the extension of the end of the ingot; and lowering the ingot at a rate sufficient to compensate for the extension thus produced so as to maintain its position just below the mold without breaking the seal formed by the slush.
- 20 7. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 25 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.
- 30 8. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 35 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.
- 40 9. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 45 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.
- 45 10. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 50 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.
- 55 11. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 60 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.
- 65 12. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 65 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.
- 70 13. The method of continuously casting ingot of alloyed magnesium having a wide freezing range which comprises maintaining the precast end of the ingot directly below and adjacent to the bottom of a short vertically disposed mold, the inside wall of said mold sloping inwardly from the bottom; continuously supplying the molten alloy to the mold so as to form a pool therein over the end of the ingot; applying a coolant to the sides of the ingot so as to carry away heat 75 from the liquid metal in the mold thereby to form a body of slush of liquid metal mixed with solid metal particles beneath the pool, the lower portion of the slush adjacent to the precast end of the ingot freezing thereto and increasing its length; continuously lowering the ingot while supplying the molten metal to the mold and vibrating the mold; and regulating the lowering rate of the ingot so that the freezing of slush thereonto occurs substantially wholly below the mold, the unfrozen portion of the slush forming a seal between the mold and the frozen slush thereby to prevent escape of liquid metal from the mold.

ADOLPH T. PETERS.